

## UNITED STATES PATENT OFFICE

EARL P. STEVENSON, OF NEWTON, AND HARRY A. BURON, OF BOSTON, MASSACHUSETTS,  
ASSIGNORS TO THE RICHARDSON COMPANY, OF LOCKLAND, OHIO, A CORPORATION  
OF OHIO

## PROCESS OF FORMING PULPS

No Drawing.

Application filed May 31, 1929. Serial No. 367,606.

Our invention relates to the preparation of pulps containing desired proportions of water insoluble binder substances and which can be felted into sheets upon conventional types of paper board and felt making machinery. Among the binder substances of the type noted are to be enumerated coal tars, asphalts, bitumens, and in general heat plastic materials. The fibrous ingredients may be any of those which, in pulp form, are suitable for paper making.

It is an object of our invention to provide a modification of the "premix process" described in our co-pending application for patent, Serial No. 314,551, filed October 23, 1928, to which reference is hereby made for a description of the ultimate product which it is desired to form. This product with respect to a particular type of binder, can be described as a bituminous, fibrous stock in aqueous suspension, wherein the asphalt or other bitumen is uniformly dispersed in the form of discrete particles having in general a globular or spherical form. This result is secured without the use of any emulsifying agent, such as colloidal clay. The discrete particles of binder substance are not rendered non-adhesive by a surface coating of an adsorbed emulsifying agent.

The present modification is primarily concerned with the mechanics of our "premixing process" above referred to, and particularly with the first step in which fibers wet with water are dispersed in a gummy or viscous binder, of which asphalt is one example. In carrying out this process it is essential to keep the fibers moistened with water during the mastication with binder substance, and thereby to prevent a complete coating of the fibers with said binder substance. It is a characteristic of such fibrous compositions that they can be dispersed in water.

The present improvement is specifically addressed to the handling of waste fibrous materials such as rags, which can not be used directly in the preferred procedure set forth in our original application, but require for adaptation thereto, a pre-treatment such as cutting, and fibration in a beater. For such products as asphalt roofing (particularly

shingles) it is deemed necessary to use a fiber furnish consisting chiefly of rag stock; and it is therefore highly desirable to provide an economical means for using rags while at the same time achieving the advantage inherent in our above referred to "premix process".

Our improved process is also directed to other ends which do not concern alone the use of a rag stock for the fiber base. One of these objects is to shorten materially the time previously required for pre-mixing a heat-fusible binder and a fibrous material to secure an association capable of ready reduction to an aqueous pulp suitable for fabrication into sheets on a paper machine.

Another object is to improve the quality of the pulp so made, by securing a more uniform distribution of binder, with particular reference to the size of particles. Yet other objects are to secure a more complete disintegration of the fibrous material used into its elementary fibers, in order thereby to minimize the time necessary for refining the ultimate pulp in either the beater or the jordan or both, to reduce the cost of "premixing" especially in the item of power, and to provide a semi-automatic operation.

Another advantage is to extend the practical application of our "premixing process" to heat fusible binders which are so viscous at temperatures readily obtainable in an open mixer and in the presence of water as to be practically unworkable therein. Examples of such binders are asphalts having a ball and ring softening point of approximately 200° F. and higher. Shellac is another such material.

In place of the open Werner-Pfleiderer mixer previously described as the preferred apparatus for premixing, a steam jacketed closed mixer fitted with a mechanically operated ram serving to close the top of the mixer and to force the charge positively into working contact with the mixing mechanism, is now recommended. Such an apparatus is exemplified by that described in the Bantbury United States Patent No. 1,200,070 dated October 3, 1916.

This type of apparatus makes it possible to effectively use a high input power, and

thereby to achieve a material shortening in the premixing time. Where thirty minutes are generally required in the open type of mixer, two to three minutes are here sufficient.

We have also discovered, when using this type of mixer, that rags can be handled directly therein. In a typical operation wet rags can be directly charged into the beater, followed by the addition of the binder, which need not be previously liquefied. A binder such as asphalt when in a viscous state, assists directly in the disintegration of the rags to a non-structural mass in which the fibers are liberated. In like manner strong fibrous structures such as heavy kraft paper, asphalt saturated and coated rag felt, partially digested wood such as sulfite tailings and the like can be utilized to advantage and with over-all economy. In some cases it may be desirable to introduce the binder before the fibrous material, though in general we prefer to reverse this procedure.

The material delivered from the above step is a more or less adhesive, gummy mass of intimately mixed binder and fibers which latter, while appearing to be completely masticated and coated by the binder, are yet in a condition for the ready assimilation of water. The step of breaking down this mass into a watery pulp may be carried on in the same mixer; but we prefer to transfer the material at this stage to another mixer. A Werner-Pfleiderer is well adapted to the next operation.

The amount of water added in the second step is immaterial as to the upper limit. Generally it will be found desirable to employ heat at this stage, though with certain types of asphalts or other binders, this may be unnecessary. In some instances the material may be added directly to a paper mill beater without resorting to this intermediate stage of pulping. Otherwise the procedure at this point is that more fully described in the co-pending application hereinabove referred to.

The advantages which are inherent in this modification of our "premix process" are attributable to mixing under a mechanically imposed pressure. In the open type of mixer the action is largely restricted to that material which at any given time is directly in contact with the mixing blades, and to that material which is passing directly between the blades and the bottom of the mixer. Power is inefficiently used in tumbling the mass around, and the filming out of the binder is not carried to a desired degree. It is to this better distribution of binder that we attribute the greater uniformity of the ultimate pulp and the more intimate association of binder and fiber which we attain.

The foregoing process is ideally adapted to the preparation of bituminous pulps.

Various types of asphalts have been successfully handled, and pulps made therewith show under the microscope spherical particles of asphalt ranging in diameter between .045 and .002 millimeters, with the average between .015 and .006 millimeters. A few of the particles may be adherent to the fibers; but the majority appear to exist as discrete particles. If the asphalt used is one that is normally adhesive, a tendency toward agglomeration may be apparent. Consequently we prefer to use asphalts which are at least semi-solid at ordinary or normal temperatures. We have successively used asphalts having a penetration as high as 30 at 77-100-5, but we prefer those slightly harder for reasons not wholly concerned with the premixing operation.

The intense mechanical operation usually results in a considerable heating of the mixer contents which will not be found disadvantageous. In the handling of certain binders it is not, therefore, necessary to apply any external heat to the mixer as through the steam jacket provided for this purpose, the internally generated heat being sufficient to cause the binder to flow under the imposed pressure. In other cases it may be found advantageous to both heat the mixer and add the binder in a molten state. This improved process of 'premixing' is not necessarily limited with respect to consistency and temperature of binder during mixing.

The resulting pulp will be utilizable in any regular paper making operation, and in the final product the binder, if it is plasticizable by heat, will be uniformly dispersed with relation to the final dried product. Sheets containing in excess of 75% of asphalt can be made more readily by this process.

Having thus described our invention, what we claim as new and desire to secure by Letters Patent, is:

1. A process of preparing a bituminous pulp, which consists in mechanically mixing wet fibrous material composed of bitumen and fiber in a closed compartment, and under pressure, and thereafter transferring said material to another mixer where it is reduced to a pulp through hydration with water assisted by a mechanical agency.

2. A process of preparing a fibrous composition capable of reduction to a pulp by mechanical agency, which consists in subjecting, under pressure, a mass of wet fibrous material and a heat plasticizable binder to the kneading action of mixing blades revolving in a closed compartment, substantially as described.

3. A process of preparing a fibrous composition capable of being felted on a screen, which comprises subjecting under heat and pressure a mass of wet cellulose fibers and a heat-fusible binder having a ball and ring softening point above 190° F., to the masti-

cating action of mixing blades revolving in a closed compartment substantially as described, while maintaining the fibers throughout the mixing cycle in a moistened condition, and thereafter reducing the resulting wet fibrous mass to a pulp by mechanical dispersion in water.

4. A process of preparing a fibrous composition capable of being felted on a screen, 10 which comprises subjecting under heat and pressure a mass of wet cellulose fibers and a bitumen having a ball and ring softening point above 190° F. to the masticating action of mixing blades revolving in a closed compartment substantially as described, while maintaining the fibers throughout the mixing cycle in a moistened condition, and thereafter reducing the resulting wet fibrous mass to a pulp by mechanical dispersion in water.

20 5. A process of preparing a fibrous composition which comprises subjecting under pressure, fibrous material and water to the mechanical action of mixing blades revolving in a closed compartment, until at least a semi-pulped mass is obtained, adding a binder, and continuing said action until a fibrous mass is obtained capable of reduction to a pulp by a mechanical agency, on the addition thereto of sufficient water.

30 6. The process of preparing a bituminous pulp from rags which consists in first adding wet rags to a closed mixer as described, adding thereto a bitumen, continuing the mixing until a substantially homogeneous mass is obtained, thereafter removing the resulting mass to another mixer, adding water and reducing said mass to the condition of a pulp suitable for handling in a beater.

7. That process of producing a pulp which 40 comprises simultaneously liberating the fibers of wetted rag stock and distributing a bitumen therethrough in minute uncoated particles, by mixing rags and bitumen in the presence of water in a closed mixer under pressure.

EARL P. STEVENSON.  
HARRY A. BURON.